

1

2,696,448

## SHRINKPROOFED WOOL AND METHOD FOR PRODUCING SAME

Irving P. Hammer, Belleville, and John B. Rust, East Hanover, N. J., assignors, by direct and mesne assignments, of one-half to Montclair Research Corporation, a corporation of New Jersey, and one-half to Ellis Foster Company, a corporation of New Jersey

No Drawing. Application March 17, 1949,  
Serial No. 82,025

32 Claims. (Cl. 117—103)

This invention relates to the treatment of wool to make it non-shrinking, while retaining its normal hand, to methods and baths for such purpose, and to the resulting treated wool products themselves, and more particularly utilizes water soluble "nylon" derivatives as agents for control of wool shrinkage.

Many suggestions for the production of shrinkproofed wool have been made in the art. But with little exception, the treated wool has not proved satisfactory either because of changes in the normal hand of the wool, or because degradation of wool fibers resulted, materially reducing wear resistance, or because material deposited in or on the wool for the purposes in hand has not been permanent enough to resist laundering, dry-cleaning, etc. The problem is distinct from that of applying relatively thick protective coatings since the wool is no longer wool of desired hand. Generally what is required is a deposit on or in the wool of relatively small amounts of materials that will prevent fibre travel usually considered to be responsible for shrinkage. Such deposit is on or under the surface of the scales of the fibers, and must accomplish the desired ends without the defects and disadvantages set forth above, giving a wool of substantially normal hand free from shrinking and felting after milling. In addition it is necessary that the methods of treating the wool be commercially feasible, i. e., that the time of treatment be reasonably short, etc.

Among the objects of the present invention is the production of shrinkproofed wool of substantially normal hand by commercially feasible processes.

Other objects include the production of such shrink-proofed wool which retains its improved characteristics resistant to laundering, dry-cleaning, etc.

Still further objects and advantages of the present invention will appear from the more detailed description set forth below it being understood that such more detailed description is given by way of illustration and explanation only, and not by way of limitation, since various changes therein may be made by those skilled in the art without departing from the scope and spirit of the present invention.

In accordance with the present invention wool while retaining its substantially normal hand, is given shrink-proof properties by the utilization of water soluble "nylon" derivatives applied by commercially feasible processes in simple treatments requiring relatively short periods of time for such treatments. Application of the water soluble "nylon" or polyamide derivatives is carried out desirably in aqueous solution followed by simple treatment to convert the water-soluble derivative into insoluble condition. Such treatment will usually be a heat treatment for drying the impregnated wool followed by a curing operation, usually heating to insolubilize the theretofore water-soluble material.

While water soluble polyamide derivatives may be used, there are several types and they are not all equivalent in that while all will give shrinkproofing, the amounts employed and the manner of application and of drying or curing will vary. With some derivatives a curing operation is essential, with other mere drying is sufficient, although curing may also be used with the latter.

The water-soluble polyamide derivatives may be applied to the wool in any desired way. The most feasible method is padding the wool with an aqueous solution of

2

the water-soluble polyamide derivative, removing excess pad liquor, and curing the impregnated wool usually with a drying step preceding curing. The amounts of water soluble polyamide derivative in the aqueous solution may 5 vary and will depend in part on the solubility of the polyamide derivative. Aqueous solutions of 1 to 25% by weight of polyamide derivatives may be used. Since it is necessary to use only very small amounts of polyamide derivative to obtain shrinkage control, the padding baths may be dilute containing for example from 10 2 to 10% by weight of the shrinkproofing agent, with baths containing 3 to 3.5% by weight desirably employed.

The impregnating step may be of the usual padding bath technique, the wool being immersed in the pad 15 liquor, and excess pad liquor removed as by squeeze rolls. The padding operation may be carried out at any temperature which causes no undesired change in the water soluble polyamide derivative at this stage. The amount of shrinkproofing agent deposited on or in the fibers or 20 the scales thereof should not be sufficient to interfere with the desired hand of the wool. Since small amounts of shrinkproofing agents are all that are needed, the end sought is easily accomplished. In general the weight increase in the wool will not exceed about 10%, although 25 it may be higher in some cases, but usually will be materially lower and may be from 2.5 to 7% by weight with preferable amounts of about 2.5 to 5% by weight.

The padded wool may then be subjected to drying for 30 removal of moisture prior to curing when the latter is used, or for insolubilizing when curing is not used. Any drying procedure may be employed provided temperatures do not reach those where the polyamide derivative is undesirably affected. Drying will usually be at temperatures below 100° C., ranges of 70-80° C. being useful, and if desired vacuum may be employed.

Curing in any desired way may be used, but usually will involve a heat treatment at elevated temperature sufficient to insolubilize the polyamide derivative. Such temperatures will usually exceed 100° C., and may desirably be in the range of from 120° to 150° C. Many of the polyamide derivatives can be subjected to much higher temperatures as for example 250 to 285° C., but such elevated temperatures are not usually desirable with treated wool products. However it should be noted that 45 the curing treatment is relatively short, for example 15 minutes at 130° C. is generally sufficient, while shorter treatments suffice at higher temperatures, for example 10 minutes at 135° C., a few minutes at 140° C., etc., so that exposures at the higher temperatures for a fraction 50 of the stated time periods will suffice, but temperatures and times of the order given in the examples below are more desirable.

Before giving exemplary procedures for the shrink-proofing operations, some considerations are given as to a preferred group of water soluble polyamide derivatives, 55 quite different from anything hitherto available in the art and particularly valuable in the production of shrink-proofed wool. These preferred derivatives are water soluble salts of disubstituted N-alkoxy methyl polyamides with carboxylic acids such as fatty acids. The nature of the substituent groups attached to nitrogen in the N-alkoxy group has been found to have an important influence on the water solubility of the stated polyamides, and as a general rule such substituent groups in the disubstituted N-alkoxy group should have less than six 60 carbon atoms.

The water soluble derivatives of the present invention are readily produced from polyamides having hydrogen bearing carbonamide groups as an integral part of the main polymer chain by reacting such polyamides with 65 a formaldehyde yielding substance and an aminoalcohol, and conversion of the resulting modified polyamide into a salt of a carboxylic acid. The treatment of the polyamide with formaldehyde for example, and aminoalcohol, may be carried out in a solution of the polyamide in a fatty acid such as formic acid, which acid will form a salt with the aminoalcohol-formaldehyde-polyamide reaction product, and to insure water solubility of such salt, the aminoalcohol used should be one which is sufficiently 70 basic to react with the fatty acid specifically with formic acid. Such desired basicity in the aminoalcohol may be

insured by the use of N-disubstituted aminoalcohols in which the substituent groups on the nitrogen are saturated aliphatic groups of less than six carbon atoms as for example alkyl groups below hexane, including methyl, ethyl, propyl, isopropyl, n-butyl, isobutyl, trimethyl methyl, and the various pentyl (amyl) groups, and such alkyl groups carrying substituent groups like hydroxy, which do not interfere with the desired water solubility. The stated water soluble salts are new entities in the art of great value since they may be used in solution in water or in aqueous emulsions. The salts per se may be recovered from the reaction medium in which they are produced by precipitation therefrom by means of an organic liquid capable of precipitating such salt from the solution in the form of a water soluble salt. The salt should not be neutralized as by addition of inorganic bases such as the caustic alkalis or ammonia, since such neutralization will destroy the water solubility of the modified polyamide.

The formation of the water soluble salt may take place by reaction of the polyamide in solution, as in formic acid, with formaldehyde and the aminoalcohol. The formaldehyde may first be reacted with the polyamide followed by reaction with the aminoalcohol, or these reactants namely polyamide, formaldehyde and aminoalcohol may be reacted simultaneously in the presence of the acid, followed by precipitation of the salt by a convenient organic solvent, and the precipitated polymer is then readily soluble in water.

The following mechanism is believed to illustrate the formation of the water soluble salt, but is offered by way of explanation only without limitation thereto, since regardless of the explanation, water soluble salts are formed. The reactions probably involve the initial reaction between the formaldehyde and the amide nitrogen to form a methylol compound. The methylol group then condenses with the hydroxy group of the N-disubstituted aminoalcohol to form an ether link. When carried out in the presence of the acid, a salt of the alkylated amine group with such acid is formed. Upon precipitation with the organic solvent, this acid salt is deposited and is soluble in water. Assuming formic acid as the acid employed, the reactions may be formulated as follows:



which forms the formic acid salt



The salt of the N-alkylated amine probably forms prior to etherification. In these formulas R is an alkylene while R<sub>1</sub> and R<sub>2</sub> are the N-disubstituent groups. While the illustrated mechanism is believed to be correct, it is not intended as limiting.

The polyamide employed may be any synthetic linear polyamide bearing recurring carbonamide groups as an integral part of the main polymer chain. The said recurring groups generally are separated by an average number of carbon atoms of at least 2. The number of such recurring groups which are modified and converted in the N-alkoxy methyl derivatives will vary with the proportions of the reactants used, but should be sufficient to yield water solubility of the salt ultimately prepared therefrom. For this purpose, generally, the recurring groups will be at least 10% of the amide groups in the main polymer chain. Extent of conversion of NH groups in the polyamides to N-alkoxy methyl groups is dependent on the anhydrous condition of the solvent (formic acid) as well as the proportions of reactants used. Thus greater conversion is obtained with 100% formic acid than with 90% formic.

The polyamide employed may be of various types, for example, a polymethylene amide of a polymethylene dicarboxylic acid, or a poly omega-amino acid, or copolymers of these polyamides just mentioned, etc. Exemplary polyamides are polyhexamethylene adipamide, polyhexamethylene sebacamide, or polymers from epsilon-

aminocaproic acid, including poly-epsilon-aminocaproic acid derived from epsilon caprolactam, copolymers such as that from ethylene diammonium sebacate and epsilon-caprolactam, etc. Generally, the molecular weight of the polymers should be rather high, that is, those which have an intrinsic viscosity above 0.4.

As to the formaldehyde reactant, any formaldehyde-yielding material may be employed. Paraform is conveniently employed. 80% aqueous formaldehyde may be used. The amount of formaldehyde is desirably from 0.5 to 2.0 parts to one part of polyamide, dependent on the extent of reaction desired.

The N-disubstituted aminoalcohol should be one capable of neutralizing formic acid. Its general characteristics have been indicated above. As exemplary of such aminoalcohols there may be mentioned alkylamines containing tertiary nitrogen, the alkylene group having for example from 1 to 4 and higher C chains. For example there may be mentioned dimethylaminoethanol, diethyl aminoethanol, methyl diethanol-amine, dimethyl isopropanolamine, triethanolamine, similar butanolamines, etc., and related compounds where the two substituents on the nitrogen may form a ring as in the morpholines such as hydroxyethyl morpholine. Certain disubstituted aminoalcohols such as phenyl diethanolamine, have a pH of about 7 (aqueous solution) and consequently are so weakly basic that they do not react sufficiently with formic acid. Therefore the "nylon" derivatives produced with such amines are either water-insoluble or only very slightly water-soluble. Other amines in this category are ethyl phenyl ethanolamine and di-2-ethyl hexyl ethanolamine. In general the molar ratio of aminoalcohol to formaldehyde will be equi-molar but may vary as from 3:1 to 1:2.

Formic acid has been particularly referred to as the reaction solvent. Other organic acids which are solvents for polyamides may be used. Carboxylic acids such as formic, acetic, hydroxyacetic, and chloroacetic, may be mentioned. Formic acid is desirably employed; and may be used in any concentration, such as 70% to 100%, in which it is a solvent for the polyamide used. Commercially available 90% formic acid may be employed conveniently.

The temperature of reaction may be any temperature at which the stated reaction takes place, for example above 30° C., but should be below that at which undesired degradation of the polyamide takes place.

The organic liquid solvent employed for precipitation of the water-soluble salt may be of any convenient solvent which gives the precipitated polymer. Acetone may be used as well as other ketones such as methyl ethyl ketone, diethyl ketone, etc.

The following examples illustrate the invention, parts being by weight unless otherwise indicated.

#### EXAMPLE A

10 parts of a poly  $\epsilon$ -amino caproic acid which has an intrinsic viscosity in meta-cresol of 0.79 was dissolved in 87 parts of 90% formic acid at 60-70° C. in a reaction flask fitted with a thermometer, stirrer and air condenser. When dissolution had occurred the solution was cooled to 30° C. by external cooling. A solution of 10 parts of paraform in 29.3 parts of diethylamino ethanol was prepared by heating the mixture until solution of the paraform was effected. The paraformdiethylaminoethanol solution was cooled to 30° C. and added dropwise to the polyamide solution with rapid stirring. During the course of the addition, dense white fumes were evolved; white salt-like particles were formed in the reaction mixture; and the temperature rose rapidly. The reaction temperature was maintained at 35-40° C. by means of a cold water bath until the dropwise addition was completed. Stirring was maintained and the reaction mixture which still contained salt-like particles, was heated to 60° C. and the reaction continued at that temperature until complete solution had occurred. The reaction was then continued at 60° C. for an additional 1/2 hour and then cooled to yield a pink fluid solution at room temperature.

45 parts of the above reaction product was treated with 158 parts of acetone with vigorous stirring to yield a faintly cloudy solution. The addition of 515 parts more acetone with constant stirring, caused the precipitation of a fibrous precipitate. The mixture was allowed to stand for 10 minutes to allow the precipitate to harden and then filtered. The filtered precipitate, still wet with acetone

and equivalent to 3.3 parts of poly  $\epsilon$ -amino caproic acid, was easily soluble in 97 parts of water at room temperature. The rate of solution in water was appreciably faster at 50-60° C. The final solution obtained had a concentration of approximately 3.3% based on the poly  $\epsilon$ -amino caproic acid.

## EXAMPLE B

10 parts of a polyhexamethylene adipamide, prepared from hexamethylene diammonium adipate, which had an intrinsic viscosity in meta-cresol of 0.47 was reacted with 87 parts of 90% formic acid, 10 parts paraform and 29.3 parts of diethylaminoethanol in the same manner as described in Example A. The reaction product was a deep red solution.

45 parts of the above solution was poured into 238 parts of acetone with vigorous stirring. A fibrous precipitate was formed which was filtered and washed with 39.5 parts of acetone. The acetone-wet precipitate, which contained the equivalent of 3.3 parts of polyhexamethylene adipamide, was dissolved in 95 parts of water at 40-50° C. with stirring. The aqueous solution was colored red.

## EXAMPLE C

10 parts of a commercial sample of polyhexamethylene adipamide which had an intrinsic viscosity in meta-cresol of 0.96 was reacted in the same fashion as described in Example A except that 137 parts of 90% formic acid was used instead of 87 parts.

57.1 parts of the final cooled reaction mixture (equivalent to 3.3 parts of the polyhexamethylene adipamide) was poured into 182 parts of acetone. A clear solution resulted. The addition of 365 parts of acetone to this solution caused the precipitation of a fibrous precipitate which was easily soluble in 97 parts of water at 60-70° C. to yield a 3.1% solution based on the original polymer.

## EXAMPLE D

10 parts of a copolymer prepared by heating 50 parts of ethylene diammonium sebacate and 50 parts of  $\epsilon$ -caprolactam under suitable conditions was reacted with 87 parts of 90% formic acid, 10 parts of paraform and 29.3 parts of diethylaminoethanol in the manner described in Example A.

Treatment of 45 parts of the above reaction mixture with 396 parts of acetone resulted in the separation of a soft gelatinous precipitate. The gelatinous material was washed several times with additional acetone by decantation which caused the precipitate to harden. The addition of 90 parts of water resulted in a clear 50 solution.

## EXAMPLE E

A solution of 10 parts of a commercial sample of a polyhexamethylene adipamide (intrinsic viscosity in meta-cresol of 0.96) was prepared in 137 parts of 90% formic acid at 60-65° C. A solution of 10 parts of paraform in 35 parts of triethanolamine was reacted with the nylon-formic acid solution employing the general procedure outlined in Example A. The reaction product was fluid at room temperature. Treatment of a portion of the above-mentioned reaction product with a large volume of acetone resulted in the separation of a fine granular precipitate which was easily soluble in water at 50-60° C.

## EXAMPLE F

A solution of 10 parts of a polyamide made from  $\epsilon$ -caprolactam (intrinsic viscosity in meta-cresol of 0.91) in 87 parts of 90% formic acid was reacted with 10 parts of paraformaldehyde and 30 parts of methyl diethanolamine employing the general procedure described in Example A. The precipitated product obtained by treating a portion of the reaction mixture with a large volume of acetone was easily soluble in water.

## EXAMPLE G

A reaction mixture was prepared from 10 parts of a polyamide made from  $\epsilon$ -caprolactam (intrinsic viscosity 0.91), 87 parts of 90% formic acid, 10 parts of paraformaldehyde, and 26 parts of dimethyl isopropanolamine by the general procedure described in Example A. The precipitated product (with acetone) was partially soluble in water at 50-60° C.

## EXAMPLE H

Example G was repeated except that the poly  $\epsilon$ -amino

5 caproic acid used had an intrinsic viscosity of 0.79 and 33 parts of hydroxyethyl morpholine instead of the dimethyl isopropanolamine. The precipitated product (with acetone) was easily soluble in water at 50-60° C. with stirring.

## EXAMPLE I

Example A was repeated except that 22 parts of dimethyl amino ethanol was used instead of the diethyl aminoethanol. The acetone precipitated derivative was 10 easily soluble in water at 40-50° C. with stirring.

The water soluble polyamide derivatives referred to above may be used as illustrated in the following examples, parts being by weight unless otherwise indicated.

## Example 1

Four lengths of 8" each were marked on a piece of wool flannel measuring 10" x 10" in size; two in the direction of the warp and two in the direction of the fill. From these measurements the area in square inches was 20 calculated. The sample was then immersed in the 3.3% aqueous solution of the poly  $\epsilon$ -amino caproic acid diethylaminoethanol derivative prepared in Example A and the excess pad liquor was removed by passing the fabric through squeeze rollers. The weight of the wool sample was noted before and after padding and from the weight increase the amount of polyamide applied to the fabric was calculated to be 3.4%. The sample was dried at 75-80° C. and then cured at 130° C. for 15 minutes.

The treated sample along with a similarly measured 30 untreated wool sample was then immersed in a 1% soap solution (1 liter) at 25° C. for a period of 2 hours. The samples were then rinsed, dried and remeasured and the "relaxation" shrinkage calculated. The samples were then laundered for 3 hours in a mechanical washing machine containing 13 liters of water at 60° C. and 35 grams of soap. The wool samples were again rinsed, dried, and remeasured and total shrinkage calculated. The area shrinkage obtained for the samples was as follows.

| Sample         | Percent Polyamide on Fabric | Relaxation Shrinkage, Percent | Total Shrinkage, Percent | Laundering Shrinkage, Percent |
|----------------|-----------------------------|-------------------------------|--------------------------|-------------------------------|
| Treated.....   | 3.4                         | 4.4                           | 5.4                      | 1.0                           |
| Untreated..... | 0.0                         | 7.7                           | 42.5                     | 34.8                          |

The finished wool sample had a dry, normal hand and good draping characteristics.

## Example 2

A sample of wool, measured as described in Example 1, was immersed in the 3.3% aqueous solution of the poly hexamethylene adipamide diethylaminoethanol derivative prepared in Example B. After the excess pad liquor was squeezed out, the weight increase of the wool indicated that the amount of polyamide applied was 3.3%. The sample was dried at 75-80° C. and cured for 15 minutes at 130° C.

60 The treated sample along with an untreated measured wool sample was subjected to "relaxation" and laundering as described in Example 1, area measurements being taken after each process. The results obtained were as follows.

| Sample         | Percent Polyamide on Fabric | Relaxation Shrinkage, Percent | Total Shrinkage, Percent | Laundering Shrinkage, Percent |
|----------------|-----------------------------|-------------------------------|--------------------------|-------------------------------|
| Treated.....   | 3.3                         | 5.0                           | 9.4                      | 4.4                           |
| Untreated..... | 0.0                         | 11.0                          | 41.4                     | 30.4                          |

The finished wool sample had a dry, normal hand and good draping characteristics.

## Example 3

A sample of wool, measured in the usual fashion, was 75 immersed in the 3.1% aqueous solution of the commercial poly hexamethylene adipamide-diethylaminoethanol derivative prepared in Example C. The weight increase of the wool sample, after the excess pad liquor was squeezed out, indicated that 2.9% of the polyamide had been applied. The sample was dried at 75° C. and cured at 130° C. for 15 minutes.

The treated sample together with untreated sample

was "relaxed" and laundered in the manner described in Example 1 except that the laundering was for 2 hours. The shrinkage data obtained was as follows:

| Sample         | Percent Polyamide on Fabric | Relaxation Shrinkage, Percent | Total Shrinkage, Percent | Laundering Shrinkage, Percent |
|----------------|-----------------------------|-------------------------------|--------------------------|-------------------------------|
| Treated.....   | 2.9                         | 4.9                           | 8.4                      | 3.5                           |
| Untreated..... | 0.0                         | 9.8                           | 37.2                     | 27.4                          |

The finished wool sample has a dry, normal hand and good draping characteristics.

#### Example 4

An aqueous solution of a commercial poly hexamethylene adipamide-triethanolamine derivative was prepared in the manner described in Example E. The concentration of the solution was 3.3%, based on the weight of the polyamide. A sample of wool, measured in the usual fashion, was immersed in the solution. The weight increase of the wool sample, after removing the excess pad liquor, indicated that 3.3% of the resin had been applied. The sample was dried at 75° C. and cured at 130° C. for 15 minutes.

The cured sample together with an untreated wool sample was "relaxed" and laundered in the manner described in Example 1 except that the laundering was for 2 hours. The shrinkage data obtained was as follows:

| Sample         | Percent Polyamide on Fabric | Relaxation Shrinkage, Percent | Total Shrinkage, Percent | Laundering Shrinkage, Percent |
|----------------|-----------------------------|-------------------------------|--------------------------|-------------------------------|
| Treated.....   | 3.3                         | 3.4                           | 3.4                      | 0.0                           |
| Untreated..... | 0.0                         | 9.8                           | 37.2                     | 27.4                          |

The finished wool sample had a dry, normal hand and good draping characteristics.

#### Example 5

An aqueous solution of a poly  $\epsilon$ -amino caproic acid-methyl diethanolamine derivative was prepared in the manner described in Example F. The concentration of the solution was 3.3% based on the weight of the polyamide. A measured sample of wool was treated with the solution in the usual fashion and subsequent to the removal of excess pad liquor, the sample was dried and cured under the same conditions as described in Example 4. The weight pick-up of the wool sample after padding indicated that 3.4% of the polyamide had been applied to the wool.

After the "relaxation" and laundering processes were carried out as described in Example 4, the shrinkage data was as follows:

| Sample         | Percent Polyamide on Fabric | Relaxation Shrinkage, Percent | Total Shrinkage, Percent | Laundering Shrinkage, Percent |
|----------------|-----------------------------|-------------------------------|--------------------------|-------------------------------|
| Treated.....   | 3.4                         | 4.9                           | 6.4                      | 1.5                           |
| Untreated..... | 0.0                         | 10.1                          | 39.2                     | 29.1                          |

The finished wool sample had a dry, normal hand and good draping characteristics.

#### Example 6

A 3.3% aqueous solution (based on the weight of the polyamide) was prepared for a poly  $\epsilon$ -amino caproic acid-dimethyl aminoethanol derivative as described in Example I. The solution was padded onto a measured sample of wool; the weight pick-up of the wool after the removal of the excess pad liquor indicated that 3.3% of the polyamide had been applied. The sample was dried, cured, relaxed and laundered by the general method described in Example 1, and the following shrinkage results were obtained:

| Sample         | Percent Polyamide on Fabric | Relaxation Shrinkage, Percent | Total Shrinkage, Percent | Laundering Shrinkage, Percent |
|----------------|-----------------------------|-------------------------------|--------------------------|-------------------------------|
| Treated.....   | 3.3                         | 7.9                           | 10.3                     | 2.4                           |
| Untreated..... | 0.0                         | 11.0                          | 41.4                     | 30.4                          |

The finished wool sample had a dry, normal hand and good draping characteristics.

In the water soluble polyamide derivatives of the type specifically emphasized above, the modified polyamide or "nylon" residue in such water soluble salts is probably the cation as the formulations given above indicate. Such derivatives are completely different in nature from water soluble polyamide derivatives where the "nylon" residue is the anion. While the cation type are particularly valuable for shrinkproofing wool, the anion type though quite different may also be employed in shrinkproofing operations and the following material is concerned with such anion types. They will for the most part fall into two general groups.

One such group is a water soluble polyamide derivative having a group or groups in the polymer chain, of the formula



in which  $\text{R}_5$  is a saturated aliphatic divalent hydrocarbon radical, such as alkylene, containing from 1 to 17 carbon atoms and  $\text{R}_6$  is a cation such as hydrogen, metals, the ammonium radical, or monovalent hydrocarbon radicals containing from 1 to 7 carbon atoms. The water soluble salts with for example alkali metals,  $\text{NH}_4$ , etc., or with complex organic ammonium groups such as quaternary trimethyl benzyl ammonium hydroxide may be used. They are produced by reacting a synthetic linear polyamide having a hydrogen bearing amide group, in the presence of an oxygen containing acid catalyst, with formaldehyde and a hydroxy carboxylic acid or an ester of a hydroxy carboxylic acid or mixtures of such acids and esters. Such reaction products may be converted into water-soluble salts where the "nylon" residue is in the anion.

The synthetic linear polyamides used may be those set forth above for the production of the cation type water soluble derivatives.

The oxygen containing acid catalysts include fatty acids and substituted fatty acids such as formic, acetic, chloroacetic, trimethyl acetic, aromatic acids such as benzoic, sulfonic acids such as p-toluene sulfonic, dibasic acids such as oxalic, maleic, etc., and even inorganic acids such as phosphoric. Such acid catalyst should have an ionization constant of at least  $9.6 \times 10^{-6}$ .

While formaldehyde has been referred to, it is generally used in the form of paraformaldehyde, but the same considerations apply here as to formaldehyde and the ratio of formaldehyde to synthetic linear polyamide as given above for the cation type water soluble salts.

The hydroxy carboxylic acids are generally the mono-hydroxy aliphatic acids of for example 2 to 17 carbon atom saturated chains, such as glycolic, lactic, 10-hydroxydecanoic, 12 hydroxy stearic, etc., although poly-hydroxy acids of this type, such as tartaric, etc., may be used. The esters are those of the stated acids with alkanols and alkoxy alkanols such as methyl, ethyl, butyl and methoxymethyl alcohols, as well as esters of cyclo-aliphatic alcohols such as cyclohexyl alcohol, and esters of aralkyl alcohols such as benzyl alcohol. It will be noted that generally the hydroxyl group is attached to an aliphatic carbon. The amounts of acid or ester will usually be determined on the formaldehyde, equi-molar ratios being preferred, but molar ratios of 1:2 to 2:1 may be used.

The reactions are carried out at any temperature from room (20° C.) to 150° C. and higher, but of course below temperatures undesirably affecting the polyamide.

The following examples illustrate these water soluble derivatives, parts being by weight unless otherwise indicated.

#### EXAMPLE J

A mixture of 50 parts polyhexamethylene adipamide (intrinsic viscosity above 0.4), 50 parts paraformaldehyde, 200 parts methyl glycolate, 7.5 parts water, and 1.7 parts 85% phosphoric acid was heated in a closed vessel with agitation to 125° C. and for 15 minutes at 125–135° C., and then cooled to room temperature rapidly. The solution obtained was diluted with 200 parts of ethanol and water (4:1 by volume) and sufficient ammonia to neutralize the phosphoric acid, and filtered. To the clear filtrate water (3000 parts) was added to precipitate the N-carbomethoxy methyl polyhexamethylene adipamide

and the latter washed with water. This product may be converted into the water soluble potassium salt by first dissolving in methanol at about 60° C. (50 parts adipamide to 100 parts methanol). Potassium hydroxide (7 parts) was added and the solution evaporated under reduced pressure to dryness. The resulting salt is readily soluble in water.

#### EXAMPLE K

175 parts of polyhexamethylene adipamide was dissolved in 700 parts of a mixture of formic acid and acetic anhydride (1.5:1) at 65° C. A suspension of 215 parts paraformaldehyde in 665 parts methyl glycolate, containing a trace of NaOH was added, and some 15 minutes later 665 parts of methyl glycolate were added and the temperature maintained at about 60° C. for about 15 minutes. The solution was poured into 3150 parts of acetone and ice cold water (4:5) and the modified polymer precipitated by addition of aqueous ammonia, and washed. The resulting N-carbomethoxy methoxy methyl polyamide may be converted to the water soluble salt by sodium hydroxide in methanol similarly to the production of the potassium salt in Example J.

Another type of water soluble polyamide derivative having the modified "nylon" residue in the anion is as follows. The polymer chain contains recurring groups of the formula



where X is oxygen or sulphur preferably but may be nitrogen or phosphorus, and R<sub>7</sub> is an organic radical containing an aliphatic carbon attached to X, said recurring groups constituting at least 10% of the amide groups in the polyamide chain, the synthetic polyamide used having an intrinsic viscosity of at least 0.4. They are prepared by reacting such a synthetic linear polyamide having hydrogen-bearing amide groups as an integral part of the main polymer chain, with formaldehyde and an alcohol or having an ionization constant of at least  $9.6 \times 10^{-6}$  as described above. Further conductance of the acid in this as in the earlier instances should be limited to acids whose conductance is not high enough to include acids like hydrochloric acid which cause degradation of the "nylon" chain.

The synthetic linear polymer used, the oxygen containing acid, and the formaldehyde are governed by the same considerations as set forth above in connection with the anion type water soluble polyamide derivatives.

The alcohol or mercaptan is one containing reactive hydrogen as determined for example by the Zerewitinoff method. Amines, sulfonamides, amides and phosphines may also be used.

The reaction may be carried out by dissolving synthetic linear polyamide in for example formic acid and reacted at moderate temperatures as for example 60-100° C. with an alcohol and formaldehyde. The ratio of formaldehyde to polyamide and of alcohol to formaldehyde may lie within the limits for analogous reactants in the other illustrated anion type water soluble polyamide derivatives.

The following example sufficiently illustrated these derivatives, parts being by weight unless otherwise indicated.

#### EXAMPLE L

15 parts of an interpolymer (intrinsic viscosity of 0.8) was dissolved in 60 parts formic acid (sp. gr. 1.20). The interpolymer was derived from hexamethylene diammonium adipate and hexamethylene diammonium sebacate (3:7). This solution was heated to 75° C. for 30 minutes with 10 parts of paraformaldehyde and 56 parts of methylhydroxy acetate. The N-carbomethoxy methoxy methyl polyamide may be precipitated by pouring the solution into aqueous sodium hydroxide. The water soluble potassium salt may be prepared by the procedure of Example J.

Any of these anion type water soluble polyamide derivatives may be used in shrinkproofing wool by the procedures set forth above in Examples 1-6 for the cation type. The same considerations as to solution concentration, weight of deposit on wool, temperature of treatment, etc., apply, as well as the considerations for drying and curing the impregnated wool. However the cation type derivatives give a better shrinkproofed product.

Having thus set forth our invention, we claim:

1. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the water soluble polyamide derivative is an acid salt of a disubstituted *N*-alkoxy methyl polyamide the polyamide being a synthetic polyamide having carbamide groups as an integral part of the main polymer chain.

2. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the polyamide derivative contains recurring groups of the formula:



where

30.  $\begin{array}{c} -O-R-N \\ | \\ R_2 \end{array}$  is the residue of aminoalcohol sufficiently basic to react with formic acid the said recurring groups being separated by an average number of carbon atoms of at least 2.
35. 3. The method of claim 2 in which R is an alkylene and R<sub>1</sub> and R<sub>2</sub> are saturated aliphatic groups of less than six carbon atoms.

45. 4. The method of claim 3 in which the N in the

50.  $\begin{array}{c} R_1 \\ | \\ -O-R-N \\ | \\ R_2 \end{array}$  is in the form of a salt with a fatty acid.
55. 5. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the impregnated wool is subjected to a drying operation by heating at a temperature not exceeding 100° C. before the curing step, and the curing step is carried out at a temperature above 100° C. but below about 150° C.
60. 6. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the water soluble polyamide derivative contains in the polymer chain a group having the formula
65.  $\begin{array}{c} -C=O \\ | \\ -N-CH_2-O-R_5COOR_6 \end{array}$

70. in which R<sub>5</sub> is a saturated aliphatic divalent hydrocarbon radical containing from 1 to 17 carbon atoms and R<sub>6</sub> is a cation selected from the group consisting of hydrogen,
75. 80.
- 85.

## 11

metals, the ammonium radical and monovalent hydrocarbon radicals containing from 1 to 7 carbon atoms.

7. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the water soluble polyamide derivative contains as an integral part of the polyamide chain recurring groups of formula



which recurring groups are separated by an average number of carbon atoms of at least 2, and in which X is selected from the group consisting of oxygen, sulphur, nitrogen and phosphorus and R<sub>7</sub> is an organic radical containing an aliphatic carbon atom attached to X said recurring groups constituting at least 10% of the amide groups in the polyamide chain.

8. The method of shrinkproofing wool by impregnating wool with a water soluble amido-N-alkoxy-substituted polyamide derivative of a synthetic polyamide which contains hydrogen-bearing amide nitrogen atoms and of intrinsic viscosity above 0.4 which derivative contains in the polymer chain a group having the formula



in which R<sub>3</sub> is a saturated aliphatic divalent hydrocarbon radical containing from 1 to 17 carbon atoms and R<sub>6</sub> is a cation selected from the group consisting of hydrogen, metals, the ammonium radical and monovalent hydrocarbon radicals containing from 1 to 7 carbon atoms, in an amount of from about 2.5 to 10% by weight on the wool insufficient to produce a continuous protective coating on the wool but sufficient to produce shrinkproofing, and drying the impregnated wool.

9. Shrinkproofed wool of substantially normal hand carrying an insolubilized deposit of a water-soluble polyamide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing in which the water-soluble polyamide derivative is an acid salt of a disubstituted -N-alkoxy methyl polyamide the polyamide being a synthetic polyamide having carbonamide groups as an integral part of the main polymer chain.

10. Shrinkproofed wool as set forth in claim 9 in which the polyamide derivative contains recurring groups of the formula



where



is the residue of aminoalcohol sufficiently basic to react with formic acid the said recurring groups being separated by an average number of carbon atoms of at least 2.

11. Shrinkproofed wool as set forth in claim 10 in which R is an alkylene and R<sub>1</sub> and R<sub>2</sub> are saturated aliphatic groups of less than six carbon atoms.

12. Shrinkproofed wool as set forth in claim 11 in which the N in the



is in the form of a salt with a fatty acid.

13. Shrinkproofed wool of substantially normal hand carrying an insolubilized deposit of a water-soluble poly-

## 12

amide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing, in which the water soluble polyamide derivative contains in the polymer chain a group having the formula



in which R<sub>5</sub> is a saturated aliphatic divalent hydrocarbon radical containing from 1 to 17 carbon atoms and R<sub>6</sub> is a cation selected from the group consisting of hydrogen, metals, the ammonium radical and monovalent hydrocarbon radicals containing from 1 to 7 carbon atoms.

14. Shrinkproofed wool of substantially normal hand carrying an insolubilized deposit of a water-soluble polyamide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing, in which the water soluble polyamide derivative contains as an integral part of the polyamide chain recurring groups of formula



which recurring groups are separated by an average number of carbon atoms of at least 2, and in which X is selected from the group consisting of oxygen, sulphur, nitrogen, and phosphorus and R<sub>7</sub> is an organic radical containing an aliphatic carbon atom attached to X, said recurring groups constituting at least 10% of the amide groups in the polyamide chain.

15. Shrinkproofed wool of substantially normal hand carrying an insolubilized deposit of a water-soluble polyamide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing, in which the polyamide is selected from the group consisting of a polymethylene amide of a polymethylene dicarboxylic acid, a poly-*e*-amino acid and interpolymers of the aforesaid specific polyamides.

16. Shrinkproofed wool of substantially normal hand carrying an insolubilized deposit of a water-soluble polyamide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing, in which the polyamide is a poly-*epsilon*-amino caproic acid.

17. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the polyamide derivative contains recurring groups of the formula



where



is the residue of aminoalcohol sufficiently basic to react with formic acid the said recurring groups being sepa-

rated by an average number of carbon atoms of at least 2, and in which the N in the



is in the form of a salt with a fatty acid.

18. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the polyamide is a polymethylene amide of a polymethylene dicarboxylic acid and the water soluble polyamide derivative is an acid salt of a disubstituted -N-alkoxy methyl polyamide the polyamide being a synthetic polyamide having carbonamide groups as an integral part of the main polymer chain, the method including drying the impregnated wool by heating at a temperature not exceeding 100° C. before the curing step, and curing at a temperature between about 100° C. and 150° C.

19. The method of claim 18 in which the polyamide derivative contains recurring groups of the formula



where



is the residue of aminoalcohol sufficiently basic to react with formic acid the said recurring groups being separated by an average number of carbon atoms of at least 2.

20. The method of claim 19 in which R is an alkylene and R<sub>1</sub> and R<sub>2</sub> are saturated aliphatic groups of less than six carbon atoms.

21. The method of claim 20 in which the N in the



is in the form of a salt with a fatty acid.

22. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the polyamide is a polymethylene amide of a polymethylene dicarboxylic acid and the water soluble polyamide derivative is an acid salt of a disubstituted -N-alkoxy methyl polyamide, the polyamide being a synthetic polyamide having carbonamide groups as an integral part of the main polymer chain, and in which the water soluble polyamide derivative contains in the polymer chain a group having the formula



in which R<sub>5</sub> is a saturated aliphatic divalent hydrocarbon radical containing from 1 to 17 carbon atoms and R<sub>6</sub> is a cation selected from the group consisting of hydrogen, metals, the ammonium radical and monovalent hydrocarbon radicals containing from 1 to 7 carbon atoms.

23. The method of shrinkproofing wool while retaining substantially normal hand by impregnating wool from an aqueous solution with from about 2.5 to 10% by weight on the wool of a water soluble polyamide derivative of a polyamide which contains hydrogen-bearing amide

nitrogen atoms of intrinsic viscosity above 0.4, said deposit being insufficient to modify the normal hand of the wool but sufficient to give shrinkproofing and curing by heating the product at a temperature below that of substantial injury to wool or polyamide derivative, in which the polyamide is a polymethylene amide of a polymethylene dicarboxylic acid and the water soluble polyamide derivative is an acid salt of a disubstituted -N-alkoxy methyl polyamide, the polyamide being a synthetic polyamide having carbonamide groups as an integral part of the main polymer chain, and in which the water soluble polyamide derivative contains as an integral part of the polyamide chain recurring groups of the formula



which recurring groups are separated by an average number of carbon atoms of at least 2, and in which X is selected from the group consisting of oxygen, sulphur, nitrogen and phosphorus and R<sub>7</sub> is an organic radical containing an aliphatic carbon atom attached to X said recurring groups constituting at least 10% of the amide groups in the polyamide chain.

24. Shrinkproofed wool of substantially normal hand carrying an insolubilized deposit of a water-soluble polyamide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing, in which the polyamide derivative contains recurring groups of the formula



where



is the residue of aminoalcohol sufficiently basic to react with formic acid the said recurring groups being separated by an average number of carbon atoms of at least 2.

25. Shrinkproofed wool as in claim 24 in which R is an alkylene and R<sub>1</sub> and R<sub>2</sub> are saturated aliphatic groups of less than six carbon atoms.

26. Shrinkproofed wool as in claim 25 in which the N in the



is in the form of a salt with a fatty acid.

27. The shrinkproofed wool of substantially normal hand carrying an insolubilized deposit of a water-soluble polyamide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing, in which the polyamide is a polymethylene amide of a polymethylene dicarboxylic acid and the water soluble polyamide derivative is an acid salt of a disubstituted -N-alkoxy methyl polyamide the polyamide being a synthetic polyamide having carbon amide groups as an integral part of the main polymer chain.

28. Shrinkproofed wool as in claim 27 in which the polyamide derivative contains recurring groups of the formula



where



85 is the residue of aminoalcohol sufficiently basic to react

15

with formic acid the said recurring groups being separated by an average number of carbon atoms of at least 2.

29. Shrinkproofed wool as in claim 28 in which R is an alkylene and R<sub>1</sub> and R<sub>2</sub> are saturated aliphatic groups of less than six carbon atoms.

30. Shrinkproofed wool as in claim 29 in which the N in the



is in the form of a salt with a fatty acid.

31. Shrinkproofed wool of substantially normal hand carrying an insolubilized deposit of a water-soluble polyamide derivative of a synthetic polyamide containing hydrogen-bearing amide nitrogen atoms and of intrinsic viscosity above 0.4, in an amount of from about 2.5 to 10% by weight on the wool insufficient to modify the normal hand of the wool substantially but sufficient to give shrinkproofing, in which the polyamide is a polymethylene amide of a polymethylene dicarboxylic acid and the water soluble polyamide derivative is an acid salt of a disubstituted -N-alkoxy methyl polyamide the polyamide being a synthetic polyamide having carbon amide groups as an integral part of the main polymer chain and the water soluble polyamide derivative contains as an integral part of the polymer chain a group having the formula



in which R<sub>5</sub> is a saturated aliphatic divalent hydrocarbon radical containing from 1 to 17 carbon atoms and R<sub>6</sub> is a cation selected from the group consisting of hydrogen, metals, the ammonium radical and monovalent hydrocarbon radicals containing from 1 to 7 carbon atoms.

32. Shrinkproofed wool of substantially normal hand

16

carrying an insolubilized deposit of a water-soluble polyamide derivative of a synthetic polyamide containing hydrogen-bearing amide nitrogen atoms and of intrinsic viscosity above 0.4, in an amount of from about 2.5 to

5 10% by weight on the wool insufficient to modify the normal hand of the wool substantially but sufficient to give shrinkproofing, in which the polyamide is a polymethylene amide of a polymethylene dicarboxylic acid and the water soluble polyamide derivative is an acid salt of a disubstituted -N-alkoxy methyl polyamide the polyamide being a synthetic polyamide having carbon amide groups as an integral part of the main polymer chain and the water soluble polyamide derivative contains as an integral part of the polyamide chain recurring groups of formula



which recurring groups are separated by an average number of carbon atoms of at least 2, and in which X is selected from the group consisting of oxygen, sulphur, nitrogen and phosphorus and R<sub>7</sub> is an organic radical containing an aliphatic carbon atom attached to X said recurring groups constituting at least 10% of the amide groups in the polyamide chain.

References Cited in the file of this patent

UNITED STATES PATENTS

| Number    | Name          | Date          |
|-----------|---------------|---------------|
| 2,347,024 | Beer          | Apr. 18, 1944 |
| 2,406,958 | McQueen       | Sept. 3, 1946 |
| 2,412,993 | Larchar       | Dec. 24, 1946 |
| 2,430,907 | Cairns        | Nov. 18, 1947 |
| 2,443,450 | Graham et al. | June 15, 1948 |
| 2,526,637 | Cupery        | Oct. 24, 1950 |